

## UNITED STATES PATENT OFFICE

2,673,183

METAL CUTTING OIL DERIVED FROM  
OXIDIZED PETROLEUM OIL

Everett C. Hughes, Shaker Heights, and David Frazier, Bay Village, Ohio, assignors to The Standard Oil Company, Cleveland, Ohio, a corporation of Ohio

No Drawing. Application August 16, 1949,  
Serial No. 110,674

13 Claims. (Cl. 252—34.7)

1

The present invention relates to a novel neutralized, oxidized oil suitable for use particularly as a cutting oil or as an additive to a cutting oil base stock, and to a process of preparing the same.

It is known generally that lard oil is included in many cutting oils now on the market. The inclusion of lard oil in such cutting oils is based on the observation that the lard oil component tends to reduce tool wear and improve the surface finish of the work. The use of lard oil as an additive cutting oil stocks has the disadvantage of involving considerable expense. This is due to the relatively high cost of the lard oil, the undependable supply thereof, the variation in the amount of free fatty acids in the available lard oil and the necessity for removing considerable foreign matter therefrom before it is suitable for blending with a cutting oil base.

The objects of the present invention are to provide an oil that is useful not only as an inexpensive substitute for the lard oil normally included in a cutting oil blend but which may also be used by itself as a cutting oil, as well as to provide a process for making such an oil and a cutting oil blend containing said oil.

It has now been found that such an oil can be obtained by first oxidizing a refined oil having an A. S. T. M. aniline point over 105°, an aromatic content below about 12%, and containing less than 0.2% total sulfur and then neutralizing it with a strong base. Examples of such light oils for oxidation are light solvent-extracted or white petroleum oil. If desired, the neutralized oil may be treated with elemental sulfur to effect a solution of sulfur in the oil.

A sulfurized oil so prepared has been found to have excellent cutting ability when used alone. When the oil of this invention, sulfurized or unsulfurized, is blended with a sulfurized cutting oil stock in a proportion upwards of about 3% by weight, or with an unsulfurized cutting oil base that is subsequently sulfurized, the resulting blend is a cutting oil of improved cutting ability that is effective in materially reducing tool wear and improving the surface finish of the work.

It is generally preferable to start with a highly refined light solvent-extracted oil having a viscosity ranging between about 75 and 150 SUS at 100° F. This oil is oxidized to a saponification number between about 20 and 80 and an A.S.T.M. neutralization number between about 12 and 25 and, when so oxidized, normally has a viscosity ranging from about 300 to about 600 SUS at 100° F. and an optical density of between 100 and 300. 55

2

The oxidation may, e. g., be effected by passing air through the oil for several hours while maintaining the oil at an elevated temperature of the order of 200° to 350° F. Processes of oxidizing oil are well known, and this step of the process is well developed art. The oxidation is usually carried out in the presence of a catalyst such as manganese naphthenate or manganese stearate. If the initial oil is less highly refined, it is usually desirable to supplement the catalyst, after the reaction has started, with a slow addition of a minor amount of a strong caustic such as sodium or potassium hydroxide or carbonate. It is important that the oxidized oil obtained in this step have a saponification number between 20 and 80. The final oil will not be soluble in the cutting oil base if the saponification number is above 80, and will not be effective in enhancing the cutting ability of a cutting oil base if the saponification number is below 20. The oxidized oil so obtained is strongly acidic, and therefore corrosive, and is not compatible with ordinary paraffin cutting oil bases.

The oxidized oil is then neutralized with a strong solid or liquid base selected from the group of alkaline earth, alkali metal and nitrogen bases. It has been found preferable to conduct the neutralization with a solid base, such as lime, but excellent results have also been obtained by the use of liquid bases such as aqueous and alcoholic potassium hydroxide, sodium hydroxide, ethylene diamine, ethanolamines and equivalent nitrogen bases.

Best results, from the point of view of compatibility of the oxidized oil with a cutting oil base, are obtained when the amount of base used is approximately equal, plus or minus 50%, to the amount corresponding to the A. S. T. M. neutralization number of the oxidized oil.

When the neutralization is carried out with a solid base, a small proportion of water is preferably first added to the oxidized oil and stirred in well to facilitate the reaction. The requisite proportion of the solid base is then added, likewise stirred in well, and the mixture is heated to 100° C. for approximately an hour.

When the neutralization is carried out with a liquid base, the required amount of liquid base is simply stirred into the oil. It is observed that the liquid base at first becomes dispersed in and emulsifies with the oxidized oil to form a milky suspension, but within a minute or so the oil becomes perceptibly warmer, much darker in color and perfectly clear.

When the oxidized oil has been neutralized

## 3

with either a solid or liquid base, any water or alcohol contained therein, such as that used to dissolve the base, may be removed by any suitable method such as by air blowing the oil at an elevated temperature, until the water or alcohol content is less than about 0.1% by weight.

Elemental sulfur may be, and preferably is, added to the oxidized and neutralized oil so produced. This is best accomplished while maintaining the oil at an elevated temperature of the order of about 60° C. so that the sulfur may readily dissolve therein. The oil is then cooled to crystallize out any excess of undissolved sulfur. Alternatively, the oxidized and neutralized oil may be added either to a sulfurized cutting oil base or to an unsulfurized cutting oil base. In the latter event it is necessary to dissolve sulfur in the unsulfurized blend.

The oxidized and neutralized oil produced in accordance with the method of this invention, whether the oil is sulfurized or not, is entirely compatible with and soluble in ordinary sulfurized and unsulfurized cutting oil stocks such as straw oils having viscosities ranging between about 75 and 150 SUS at 100° F. It has an A. S. T. M. neutralization number between +1.0 and -2.0, contains less than 0.1% "water in oil," by A. S. T. M. and is soluble and stable at 10% in a neutral paraffin oil having a viscosity of 100 SUS at 100° F.

With a given cutting oil stock, sulfurized before or after the blending thereof with oxidized oil, it has been found that concentrations of the oxidized oil of this invention in amounts ranging from about 8 to about 50% by weight are optimum for reducing the wear, and therefore increasing the life of, a cutting tool. Concentrations as low as about 3% and as high as 100%, i. e., the sulfurized composition itself without any cutting oil base, have, however, been found to equal or to be superior to the best known sulfurized cutting oils available on the market.

One of the advantages of the present invention is that it provides an inexpensive, abundant and reliable source of cutting oil additive which, when blended with any known cutting oil base, imparts to it the desirable property of greatly prolonging the life of a cutting tool.

Another advantage of the invention is that it provides a simple and easily controlled method for producing a sulfurized oil that is not only superior when used in place of lard oil but may be used by itself as a cutting oil.

These and other advantages as well as the utility of the invention will become more apparent from the following examples.

## Example 1

A light solvent-extracted oil having a viscosity of 115 SUS at 100° F. was oxidized with air to a saponification number of 58 and a neutralization number of 18. The oxidized oil was neutralized by adding 1% by weight of water, which was stirred in well, and the subsequent addition of 2% by weight of lime, which was likewise stirred in well. The mixture was heated to 100° C. for one hour and then blown with air for an additional hour while maintained at 100° C. The neutralized oil was allowed to cool and settle.

The oxidized oil so neutralized was found to be compatible with paraffin oils and to form a clear solution when 20 parts thereof are mixed with 80 parts sulfurized straw paraffin oil having a viscosity of 100 SUS at 100° F. and containing 1% sulfur.

## 4

## Example 2

A solvent-extracted oil similar to that treated in Example 1 was oxidized with air to a saponification number of 47 and a neutralization number of 15 and then neutralized in substantially the same manner with 3% by weight of lime. The neutralized oil thus obtained was blown with air as in Example 1 and was found to exhibit physical properties similar to those of the oil produced in accordance with Example 1. 20 parts of the neutralized oil were blended with 80 parts of a sulfurized straw paraffin oil having a viscosity of 100 SUS at 100° F. and containing 1.2% of sulfur.

## Example 3

A light solvent-extracted oil similar to that treated in accordance with Example 1 was oxidized with air to a saponification number of 53 and a neutralization number of 13. A stoichiometric amount of potassium hydroxide in water, as indicated by the neutralization number of the oxidized oil, was then stirred into the oil so oxidized. This resulted at first in a milky suspension which was resolved after a minute or two and became perfectly clear. The oil thus neutralized was blown with air for 1/2 hour and the oil was maintained at a temperature of 100° C.

The resulting oil was found to be compatible with straw paraffin oil. A blend of 16 parts neutralized oil and 84 parts straw oil was saturated with sulfur by heating with excess sulfur. The excess sulfur crystallized out and was filtered off.

The mixture contained 1.7% sulfur.

## Example 4

A light solvent-extracted oil similar to that treated in Example 1 was oxidized to a saponification number of 60 and a neutralization number of 18. A stoichiometric excess of 60% potassium hydroxide in water was stirred into the oil so oxidized. The reaction appeared to be approximately the same as described in Example 3 except that the neutralized oil became darker and more viscous, apparently due to the excess potassium hydroxide. This oil was blown with air and 0.75% by weight of elemental sulfur was dissolved therein by saturating the oil with sulfur at 60° C. and then cooling to crystallize out the excess sulfur.

## Example 5

The method of Example 4 was repeated with the exception that initial oil was oxidized to a neutralization number 17 and the oxidized oil was neutralized with a 30% solution of potassium hydroxide in methanol and 0.7% by weight of sulfur was dissolved in the neutralized oil.

The oil blends prepared in Examples 1 to 3, 60 and the neutralized oils prepared in Examples 4 and 5, alone and in various concentrations as additives to paraffin straw oil having a viscosity of 100 SUS at 100° F. and sulfurized to a sulfur content of 1.7%, were field tested on an automatic drill milling machine to determine their effect upon tool life.

In each test, the work piece was 1/2" stock of regular "Momax HS" steel. Both flutes, having a spiral of 22°, were milled simultaneously, then indexed to a second position where both margins were clearance milled. The mechanical factors of the flute mill were: 0.218" depth on both sides, 1.625" per minute feed, 176 surface feet per minute speed, and 20-toothed cutters.

The normal tool life expectancy on this ma-

chine, under the same conditions and with the use of one of the best cutting oils on the market, made by dissolving 1% by weight of sulfur in 20% lard oil and 80% paraffin straw oil having a viscosity of 100 SUS at 100° F., is from 36 to 39 drills.

The results are listed in the table below:

| Test No. | Oil of Example | Concentration, in percent by weight of oxidized oil in cutting oil composition | Cutter Life |
|----------|----------------|--------------------------------------------------------------------------------|-------------|
| 1        | 1              | 20                                                                             | 67          |
| 2        | 2              | 16                                                                             | 60.2        |
| 3        | 3              | 16                                                                             | 49.2        |
| 4        | 4              | 50                                                                             | 46          |
| 5        | 5              | 100                                                                            | 37          |
| 6        | 5              | 33                                                                             | 51          |
| 7        | 5              | 16                                                                             | 59          |
| 8        | 5              | 8                                                                              | 51          |
| 9        | 5              | 4                                                                              | 43.4        |

In all instances it is to be noted that the tool life is above the normal expectancy when a cutting oil made in accordance with the invention is used.

A similar test but using paraffin straw oil having a viscosity of 100 SUS at 100° F. and sulfurized to a sulfur content of 1.7%, without the addition of an oxidized and neutralized oil, resulted in a cutter life of only 27.4.

Another test, conducted with a 16% concentration of an oxidized and neutralized oil prepared as in Example 5 but containing no sulfur, in paraffin straw oil likewise containing no sulfur, resulted in a cutter life of 0.

These tests show that sulfurized cutting oil bases containing widely varying concentrations of oxidized and neutralized oils prepared in accordance with the present invention are superior, in prolonging the life of cutting tools, to a cutting oil that is among the best available on the market at the present time. The tests also show that the removal of water from the oxidized oil is desirable, that sulfur is a necessary component in the oxidized oil when it is used alone, and in the blend, that optimum results are obtained when the concentration of the oxidized oil in the base ranges between about 8% and 50%, and that neutralization with a solid base gives somewhat better results than neutralization with a liquid base.

The term "optical density" in the present disclosure represents the standard logarithmic ratio of intensity of an incident ray falling on a transparent or translucent medium to the intensity of the transmitted ray for a sample length of one meter and light of wave length from 5,100 to 5,500 Angstroms.

It is to be understood that innumerable variations and modifications will immediately become apparent to those skilled in the art upon reading the foregoing disclosure. The invention contemplates all such variations and modifications as come within the scope of the appended claims.

We claim:

1. A method of making a cutting oil blend which comprises oxidizing a light solvent-extracted mineral oil to a saponification number between about 20 and 80, neutralizing the oxidized oil with a base, volatilizing the amount of any water and alcohol contained therein to reduce the amount of water and alcohol to less than about 0.1%, dissolving sulfur in said oil, and blending said oxidized and neutralized oil with a sulfurized cutting oil base stock.

2. A method of making a cutting oil which comprises oxidizing a solvent refined light mineral oil having an A. S. T. M. aniline point over 105° C., an aromatic content below about 12%, and containing less than 0.2% total sulfur, to a saponification number between about 20 and 80, neutralizing the oxidized oil with a base, substantially volatilizing any water and alcohol contained therein, and dissolving sulfur in said oil.

5 3. A method of making a cutting oil which comprises oxidizing a light solvent-extracted mineral oil to a saponification number between about 20 and 80, neutralizing the oxidized oil with a base, substantially volatilizing any water and alcohol contained therein, and dissolving sulfur in said oil.

10 4. A neutralized, oxidized, solvent refined, light mineral oil substantially free of water and alcohol and containing dissolved elemental sulfur, said neutralized, oxidized oil having, before neutralization, a saponification number between about 20 and 80 and having been neutralized with a base.

15 5. A cutting oil comprising a mineral oil base stock and at least about 3% by weight of a neutralized, oxidized, solvent refined, light mineral oil that is substantially free of water and alcohol, at least one of said components having elemental sulfur dissolved therein and said neutralized, oxidized oil component having, before neutralization, a saponification number between about 20 and 80 and having been neutralized with a base.

20 6. A cutting oil comprising a sulfurized mineral oil base stock and at least about 3% by weight of a neutralized, oxidized, solvent refined, light mineral oil substantially saturated with dissolved sulfur, said neutralized, oxidized oil being substantially free from water and alcohol and having, before neutralization, a saponification number between about 20 and 80 and having been neutralized with a base.

25 7. A cutting oil comprising a sulfurized mineral oil base stock and at least about 3% by weight of a neutralized, oxidized, solvent refined, light mineral oil that is substantially free of water and alcohol, said neutralized, oxidized oil component having, before neutralization, a saponification number between about 20 and 80 and having been neutralized with a base.

30 8. A cutting oil comprising a mineral oil base stock and at least about 3% by weight of a neutralized, oxidized, solvent refined, light mineral oil that is substantially free of water and alcohol, said neutralized, oxidized oil component having, before neutralization, a saponification number between about 20 and 80 and having been neutralized with a base, said blend having elemental sulfur dissolved therein.

35 9. In a method of making a cutting oil composition comprising an essentially two-component blend of neutralized, oxidized oil with a mineral cutting oil base stock, said blend having elemental sulfur dissolved therein, the steps which comprise oxidizing a solvent refined, light mineral oil having an A. S. T. M. aniline point over 105° C., an

40 aromatic content below about 12% and containing less than 0.2% total sulfur to a saponification number between about 20 and 80, neutralizing the oxidized oil with a base, substantially volatilizing any water and alcohol contained in the neutralized, oxidized oil, blending it with a mineral cutting oil base stock, and dissolving elemental sulfur in at least one of the components of said cutting oil composition before blending or in the blended composition.

45 75 10. The method defined in claim 9 wherein the

elemental sulfur is dissolved in the mineral cutting oil base stock before blending said component with the neutralized, oxidized oil.

11. The method defined in claim 9 wherein the elemental sulfur is dissolved in the neutralized, oxidized oil before blending said component with the mineral cutting oil base stock.

12. The method defined in claim 9 wherein the elemental sulfur is dissolved in both the neutralized, oxidized oil and the mineral cutting oil base stock before they are blended.

13. The method defined in claim 9 wherein the elemental sulfur is dissolved in the blend after blending of the neutralized, oxidized oil component with a mineral cutting oil stock.

EVERETT C. HUGHES.  
DAVID FRAZIER.

References Cited in the file of this patent  
UNITED STATES PATENTS

| Number       | Name       | Date           |
|--------------|------------|----------------|
| 1,767,147    | MacCoull   | June 24, 1930  |
| 1,863,004    | Burwell    | June 14, 1932  |
| 1,904,065    | Mackenzie  | Apr. 18, 1933  |
| 1,987,397    | Gallworthy | Jan. 8, 1935   |
| 2,121,151    | Karns      | June 21, 1938  |
| 2,142,916    | Parkhurst  | Jan. 3, 1939   |
| 2,222,643    | Zimmer     | Nov. 26, 1940  |
| 2,246,281    | Zimmer     | June 17, 1941  |
| 2,252,132    | Morway     | Aug. 12, 1941  |
| 2,257,328    | Bray       | Sept. 30, 1941 |
| 15 2,367,435 | Ruedrick   | Jan. 16, 1945  |
| 2,396,345    | Rogers     | Mar. 12, 1946  |

## FOREIGN PATENTS

| Number     | Country       | Date           |
|------------|---------------|----------------|
| 20 335,152 | Great Britain | Sept. 10, 1930 |